

## UNITED STATES PATENT OFFICE

2,192,219

## SIZING OF CELLULOSE ETHER AND ESTER MATERIALS

Herman S. Bosland, Paterson, N. J., assignor to  
Stein, Hall & Company, Inc., New York, N. Y.,  
a corporation of New York

No Drawing. Application June 14, 1937,  
Serial No. 148,113

9 Claims. (CL 134—23)

This invention relates to the treatment of cellulose ether and ester materials and more particularly to the sizing of cellulose acetate materials prior to weaving.

- 5 The sizing of certain textile materials with starch or starch derivatives presents special problems, particularly in the sizing of regenerated cellulose and cellulose ether and ester materials. Thus, in sizing regenerated cellulose an 10 ordinary starch size adheres so well to the material that a distinct problem is encountered in desizing the material after weaving. In other words, there appears to be a bond or affinity between a starch size and a regenerated cellulose. 15 On the other hand, fibers such as the well known cellulose acetate when sized with ordinary amylose sizing compositions fail to weave properly, the size being rapidly removed from the fibers under the chafing action of weaving. For 20 this reason it has not been possible to satisfactorily size cellulose ester yarns such as cellulose acetate with amylose products, and it has been necessary to rely entirely upon special sizes, particularly sizes of a protein nature such 25 as gelatin, casein and the like.
- It is an object of this invention to provide a method of sizing cellulose acetate and other cellulose ester or cellulose ether materials utilizing amylose materials. A further object is the 30 preparation of improved cellulose acetate sizing compositions. Another object is to prepare cellulose acetate sized with a composition which strengthens the fibers to resist the mechanical action of the loom and is not rapidly removed 35 under the chafing action of weaving. Other objects will appear hereinafter.

These objects are accomplished in accordance with this invention by incorporating about 20% to 25% or more of urea in a specially prepared 40 starch derivative and applying the resultant composition as a sizing composition to cellulose ester or ether fibers, particularly cellulose acetate. I have found that such a sizing composition becomes bound to cellulose acetate fibers, 45 that is, it shows a natural affinity previously lacking. The exact nature of this action is unknown, but it seems to be due to some coordinate valence bonding between the starch on the one hand and the cellulose ester on the other. 50 Good results can be obtained with compositions containing a minor proportion of urea and a major proportion of a dispersible amylose material, the amount of urea preferably being about 25% to 75% by weight of the amylose material.

The manner in which the invention may be practiced will be illustrated, but is not limited, by the following example in which the quantities are stated in parts by weight:

## Example

A sizing composition was prepared by mixing together 10 parts of a modified starch, 2 to 6 parts of urea, and 40 to 80 parts of water, and heating the mixture at a temperature of about 180° F. with agitation for 15 minutes.

A cellulose acetate yarn was then sized by the skein method by immersing it in the resultant sizing composition at a temperature of about 140° to about 150° F. If desired, the sizing may 15 be effected in the cold at temperatures of say 60° to 80° F.

The size strengthened the fibers to resist the mechanical action of the loom and was not rapidly removed under the chafing action of weaving. After weaving the size was readily removable by washing with water.

In the above example auxiliary agents may be added to the composition, for instance, 1.5 parts of glycerine or 3 parts of Turkey red. This 20 formula can be used for both skein and warp sizing.

In a similar manner other compositions may be prepared in accordance with the invention, with varying proportions of urea and amylose matter. It is usually preferable to employ a starch degeneration product, by which is meant a derivative of starch such as may be obtained by the various processes of making thin-boiling and so-called soluble starches and dextrans. By 30 a specially modified starch is meant a starch degeneration product which, after having been colloidally dispersed in water, yields a dried protective film of suitable physical characteristics for the purpose involved. In order to obtain 40 these characteristics and to form so-called solutions suitable for textile application, ordinary undegenerated starch is suitably degenerated in part, or modified, by various chemical and heat treatments. If desired, mixtures of undegenerated starch and modified starches may be used 45 in conjunction with the urea.

The term "amylose material" is employed herein to cover starch and starch derivatives or degeneration products. The expression "starch degeneration products" is employed to cover dextrans as well as modified starches. Among the suitable starchy materials may be mentioned wheat, rye, barley, oat, rice, maize and potato starches, sago and cassava flours and starch de- 55

generation products thereof, and other starches and flours, and derivatives thereof.

The proportions and concentrations of materials may vary depending upon the nature of the ingredients of the composition and other related factors. In the sizing composition of the invention for the treatment of cellulose acetate or other cellulose ester or ether materials, I prefer to use a sizing composition having a ratio of 10 solids to water within the range of about 2:5 to about 1:7.

The amount of such material incorporated into or applied to the cellulose acetate is subject to variation, but ordinarily good results are obtained 15 by adding to the cellulose acetate about 4% to about 6% of the sizing composition based upon the normally air-dry weight of the sized material. The amount of sizing composition retained by the material treated will depend largely upon 20 the concentration of the bath and the time of treatment. Ordinarily the bath may be either hot or cold. The method of treatment may be the warp method, skein method or any other suitable method.

25 It will be recognized that a wide variety of auxiliary agents may be added to the sizing compositions herein described. Among such addition agents may be mentioned fullers earth, bentonite, wetting, penetrating and dispersing agents, for 30 example, sulfonated oils, higher alcohol sulfates (e. g., dodecyl sulfate, cetyl sulfate, and similar compounds), diethylene glycol, glycerine and related substances. The proportions of these materials may also vary, depending upon the type of 35 treatment and the material treated. For instance, it is usually preferable to use about 2 parts of glycerine or 4 parts of Turkey red oil for each 80 parts of sizing composition in the treatment of cellulose acetate materials. It will be observed 40 that applicant's compositions are of such a nature as to be permanently water dispersible even upon the application of heat.

In preparing the sizing compositions described above it is preferable to prepare a dry blend of 45 amyloseous binding agent and urea as a base material. This blend is marketed in dry or powdered form and requires only the addition of water and mixing, preferably with heating, to produce the sizing composition. Auxiliary materials such as those mentioned above may also be 50 included in the dry base.

55 It will be apparent that the use of an amyloseous material intimately dispersed with urea in sizing textile fibers such as cellulose acetate has many advantages over the use of the amyloseous substance or urea per se. Starchy materials alone have not proven satisfactory in cellulose acetate sizing because of the lack of affinity with cellulose acetate. Urea has been suggested for 60 use in conjunction with starch and other materials in veneer glues but has not heretofore been applied to starch sizing mixtures for cellulose acetate and similar materials. Urea solutions have also been used to reduce the inflammability

of materials, but the use of urea alone does not fulfill the function of the combination of urea and starch or starch degeneration products for the treatment of cellulose acetate and similar materials as herein described.

Having thus described the invention, what I claim as new, and desire to secure by Letters Patent of the United States is:

1. In the art of sizing cellulose ether and ester materials, the step which comprises applying to 10 said materials a permanently water dispersible composition containing an intimate dispersion of an amyloseous substance and urea, the amount of urea being at least about 20% by weight of the amyloseous substance. 15

2. A method of sizing cellulose acetate yarn which comprises treating the yarn with a permanently water dispersible intimate dispersion of an amyloseous substance and urea in water, the amount of urea being at least about 20% by 20 weight of the amyloseous substance and the ratio of solids to water being within the range of about 2:5 to about 1:7.

3. A method of sizing cellulose acetate yarn which consists in treating the yarn with an intimate dispersion consisting essentially of about 25 10 parts of a modified starch, 2 to 6 parts of urea and 40 to 80 parts of water.

4. A cellulose acetate sizing composition comprising a permanently water dispersible intimate 30 dispersion of an amyloseous substance and urea in water.

5. A cellulose acetate sizing composition comprising a permanently water dispersible intimate dispersion of a starch degeneration product and 35 urea in water, the amount of urea being about 25% to about 75% by weight of the starch degeneration product and the ratio of solids to water being within the range of about 2:5 to about 1:7. 40

6. A sizing composition adapted for sizing cellulose acetate fibers prior to weaving and consisting essentially of an intimate dispersion of about 10 parts of a modified starch and about 2 to about 6 parts of urea in about 40 to about 80 45 parts of water.

7. A cellulose ether and ester material sized with a permanently water dispersible intimate dispersion of an amyloseous substance and urea in water. 50

8. A cellulose acetate material containing a sizing composition consisting essentially of a major proportion of amyloseous substance and a minor proportion of urea, the amount of urea being at least 25% by weight of the amyloseous 55 substance.

9. A cellulose acetate material containing a permanently water dispersible sizing composition having an amyloseous material as its sole or substantially its sole binding agent and containing 60 urea in an amount from about 25% to about 75% by weight of the amyloseous material.

HERMAN S. BOSLAND.

CERTIFICATE OF CORRECTION.

Patent No. 2,197,219.

March 5, 1940.

HERMAN S. BOSLAND.

It is hereby certified that error appears in the printed specification of the above numbered patent requiring correction as follows: Page 1, first column, line 32, for "ecetate" read acetate; and second column, line 25, after the word "red" insert oil; and that the said Letters Patent should be read with this correction therein that the same may conform to the record of the case in the Patent Office.

Signed and sealed this 9th day of April, A. D. 1940.

(Seal)

Henry Van Arsdale,  
Acting Commissioner of Patents.